

P. REMER.

PROCESS OF LIMING AND DEHAIRING HIDES.

APPLICATION FILED JUNE 14, 1918.

1,331,723.

Patented Feb. 24, 1920



Witnesses

Mary V. Spaulding

Inventor,

Peter Remer,

By Offield, Towle, Graves & Doane,  
Attorneys

# UNITED STATES PATENT OFFICE.

PETER REMER, OF MILWAUKEE, WISCONSIN, ASSIGNOR OF ONE-THIRD TO ANDREAS G. WACKENREUTER AND ONE-THIRD TO WILLIAM S. SHAW, BOTH OF CHICAGO, ILLINOIS.

## PROCESS OF LIMING AND DEHAIRING HIDES.

1,331,723.

Specification of Letters Patent. Patented Feb. 24, 1920.

Application filed June 14, 1918. Serial No. 240,009.

*To all whom it may concern:*

Be it known that I, PETER REMER, a subject of the King of Austria-Hungary, residing at Milwaukee, in the county of Milwaukee and State of Wisconsin, have invented 5 certain new and useful Improvements in Processes of Liming and Dehairing Hides, of which the following is a specification.

This invention relates to a new and improved process of liming and dehairing hides, and it has for its salient objects to put the hides in such condition upon the completing of the liming and dehairing process that they will assimilate the tanning and tan more rapidly and uniformly than heretofore; to put the dehaired hides in such condition that they will absorb or assimilate more tanning and filler; to plump or swell the hides as a result of the liming and 15 dehairing process with all of the advantages which result from so doing; to provide an inexpensive, rapid and reliable process of liming and dehairing; and in general, to provide an improved process of the character referred to.

My improved process may be carried out by the aid of any suitable series of tanks or receptacles adapted to hold the hides and liquid, and in the use of which the hides 20 can be transferred from one receptacle to the next in one direction while the treating liquid is transferred from one receptacle to the next progressively in the opposite direction.

Accordingly I have shown the apparatus in a merely diagrammatic way, since apparatus suitable for carrying out the process is well known to those skilled in the art.

In the drawing the single figure shows a 25 plan view of a series of liming vats connected with each other by suitable pipes through which the liquid may flow from one vat to the next.

In the preferred way of carrying out my improved process, I employ a series of nine vats; that number being accordingly shown in the drawing. The first and last vats of the series are utilized for preliminary and final washings, respectively, which washings 30 are not strictly parts of the process. Accordingly for convenience of description I designate the first vat *a*; number the intermediate vats 1 to 7, and designate the final

washing vat as *b*; the hides being placed in No. 1 at the start, and transferred progressively down the line. The characteristic feature of my process resides in treating the hides initially in a bath composed of water, limewater and sulfid of sodium in solution. Another important characteristic of my 55 process resides in treating the hides in the final stages of the process with limewater only, and utilizing this same limewater in forming the combined sulfid and limewater baths used in the earlier stages of the treatment, whereby the strength of the limewater is reduced and its action in combination with the sulfid improved.

Describing a preferred way of carrying out my process, I first prepare the liquor for 70 the various vats as follows:

Vats Nos. 7, 6, 5 and 4 are charged with a solution of limewater; vat No. 7 being charged with the fresh solution about 18° barkometer strong, vats Nos. 6, 5 and 4 may 75 be initially charged with solutions which are progressively weaker. In the subsequent working of the process the limewater is transferred from one to the other, and thus becomes weaker in the successive baths.

Vat No. 3 is charged with simple water, which will be changed as often as necessary to insure its operating effectively to wash out the chemical solution remaining in the 80 hides as a result of their previous treatments.

Vats Nos. 2 and 1 are charged with a solution of limewater and sulfid of sodium. The limewater of vat No. 2 is the same limewater which was used in vat No. 4, from which it 90 is transferred, and to this limewater is added from one-half to one pound of sulfid of sodium for each hide. The liquor in vat No. 1 is, in the regular working of the process, that which has been transferred from vat No. 95 2, unmodified except by the change effected by its operation upon the hides. Initially the liquors for vats No. 1 and No. 2 may be prepared of a very weak solution of lime, to which is added the stated amount of sulfid of sodium, *i.e.*, from one-half to one pound per hide.

Describing the successive steps or stages of the process, the hides are first preliminarily soaked in vat *a* until they are thoroughly softened, as usual. They are next

transferred to vat No. 1 and allowed to remain therein about one day more or less; being moved about in the vat from time to time as usual to insure uniformity of treatment. The hides are next transferred to vat No. 2 and therein treated in the same way and for approximately the same time as in vat No. 1. Next they are transferred to the washing vat No. 3 and thoroughly washed in clear water. This washing is for the purpose of eliminating the sodium sulfid charged liquor as thoroughly as practicable, since there is a tendency to produce a precipitate in and upon the hides if the latter are passed into the stronger lime baths before being properly washed free of this solution. The thorough rinsing off of the sulfid solution may be ordinarily accomplished in a short time, say from twenty minutes to a couple of hours.

From the washing vat No. 3 the hides are transferred to vat No. 4, treated therein for a period of approximately twenty-four hours, then transferred successively to vats Nos. 5, 6 and 7, in each of which they are treated for approximately twenty-four hours, and finally they are thoroughly washed out in warm water in vat designated 3. The final washing is, of course, designed to free the hides entirely of the limewater solution to which they have been subjected.

It will be noted that in preparing and transferring the liquors from vat to vat, as suggested, the limewater contained in vat No. 7 is made as a fresh charge for each batch of hides, and so also the lime and sulfid solution of vat No. 2 is replenished with the sulfid of sodium after the treatment of each batch of hides. Accordingly, after a batch of hides has been taken out of vat No. 1, the liquor of that vat is drained off and the liquor previously contained in vat No. 2 transferred through the connecting pipe 10, controlled by the turncock or valve 11. The limewater contained in vat No. 4 is next transferred to vat No. 2 through the pipe 12 and the requisite amount of sulfid of sodium added to it. The charges in vats Nos. 5, 6 and 7 are next respectively transferred to the next lower vat, and a freshly made charge of limewater charged into vat No. 7. The hides are now treated in the succession of vats as hereinbefore described.

It will, of course, be obvious that the details of treatment may be somewhat varied without departing from the spirit of my invention, and as well also the solution may be varied.

Hides which have been subjected to my improved liming process are extremely plump, and the pores thereof expanded and opened up so that the hide material is highly absorbent. As a result of this the hides quickly absorb the tanning solution to which they are afterward subjected, with

the result that the tanning proper is greatly expedited. Moreover, the plump and porous condition of the hides facilitates the absorption of an increased percentage of so-called filler, with the result of increasing 70 the body and weight of the tanned leather. Hides treated with my improved liming process are characterized by an unusual degree of softness and freedom from harmful effects due to liming.

I claim as my invention:

1. The improved process of liming hides, which consists in first soaking the hides in a hydrous solution, weak in lime and mild in sodium sulfid, then washing, and thereafter soaking the hides in materially stronger limewater unmixed with sodium sulfid.

2. The improved process of liming hides, which consists in first soaking the hides in a weaker solution of lime and sodium sulfid, then in a stronger solution of lime and sodium sulfid, then washing the hides free from the sulfid-charged liquor, and thereafter soaking in limewater.

3. The improved process of liming hides, which consists in first soaking the hides in a weaker solution of lime and sodium sulfid, then in a stronger solution of lime and sulfid, then freeing the hides of the sodium sulfid, thereafter soaking in a weaker solution of limewater, and then soaking in a stronger solution of limewater.

4. The improved process of liming hides, which consists in first soaking the hides in a solution of water, lime and sodium sulfid of moderate strength both as to the sodium sulfid and lime contents, thereafter soaking the hides in a solution of water, lime and sodium sulfid stronger than the preceding bath, then washing the hides free of the sulfid-charged liquor, and thereafter subjecting the hides to soaking treatments in a plurality of baths of limewater, each successively stronger.

5. The improved process of liming hides, which consists in passing the hides progressively through a series of treatment vats in a definite direction, soaking the hides for a substantial period in each of said treatment vats, concurrently with the transfer of the hides from vat to vat, transferring the treatment liquor successively from vat to vat in the direction opposite that of the progress of the hides; the hides being treated in the earlier stages in a solution of water, lime and sulfid of sodium, treated in the later stages in a solution of lime only, and freed from the sulfid-charged liquor between said early stage and later stage treatments.

6. The improved process of liming hides, which consists in passing the hides progressively through two series of treatment vats and soaking the hides for a substantial period in each treatment vat, the vats of 130

the first series each containing a solution of lime and sulfid of sodium; the vats of the second series containing a solution of lime only, transferring the treating solutions of each series from vat to vat of that series in the direction opposite that of the progress of the hides and adding fresh solutions

to the vats so emptied, whereby the hides are treated in successively stronger solutions in each series, and washing the hides <sup>10</sup> in water between treatments by the first and second series.

PETER REMER.